

## UNITED STATES PATENT OFFICE

2,142,835

## LEAD ALLOYS

Jesse O. Betterton, Metuchen, Albert J. Phillips, Plainfield, and Albert A. Smith, Jr., Metuchen, N. J., assignors to American Smelting and Refining Company, New York, N. Y., a corporation of New Jersey

No Drawing. Application March 19, 1937,  
Serial No. 131,860

5 Claims. (Cl. 75—167)

This invention relates to lead alloys and provides certain new and novel lead alloy compositions which, by reason of the properties they possess and exhibit, are definitely superior for use in the manufacture of such lead products as cable sheathing, grid metal, etc.

Broadly speaking, the invention may be said to provide ternary alloys of lead, calcium and magnesium possessing certain highly beneficial physical properties, and alloys comprising the base alloy of lead, calcium and magnesium with at least one additional alloying constituent imparting further desired properties to the alloy while at the same time retaining or enhancing the beneficial physical properties possessed by the base alloy itself.

More specifically, the invention provides alloys of lead, calcium and magnesium in which the combined calcium and magnesium content does not substantially exceed 0.4% of the alloy with the magnesium content being within the approximate limits of one quarter to three times the calcium content. While 0.03% to 0.05% each of calcium and magnesium is preferred, compositions containing magnesium and calcium within the limits of 0.01% to 0.3% and 0.01% to 0.1%, respectively, may be employed.

Among metals which may be added to the lead-magnesium-calcium composition are cadmium, copper, mercury and tin, all of which modify the behavior of the alloy under corrosive influences without adversely affecting the fundamental physical nature of the ternary alloy. In addition, copper stiffens the alloy moderately and accelerates its aging; mercury improves its lustre and to a moderate extent its casting properties; tin slightly improves its fluidity and casting properties. The amount of modifying or improvement metal which may be incorporated should fall within the approximate limits of 0.03% to 3% with a minimum of about three or four times the magnesium content.

The superior properties exhibited by the alloys of the invention are best shown by the following data comparing same with several of the conven-

tional alloy compositions available and often recommended for various specific purposes:

## Brinell hardness

| Material tested                           | Lead alloyed with— |         |                 |
|-------------------------------------------|--------------------|---------|-----------------|
|                                           | 8% Sb              | .05% Ca | .03% Mg-.05% Ca |
| Castings $\frac{3}{16}$ " thick.....      | 12.1               | 7.0     | 5.2             |
| Above aged 21 days at 30° C.....          | 12.9               | 8.0     | 13.4            |
| Same heated 2 hours at 100° C.....        | 13.4               | 9.5     | 15.4            |
| Grid castings $\frac{3}{16}$ " thick..... | 11.8               | 5.0     | 5.0             |
| Above aged 21 days at 30° C.....          | 13.8               | 11.4    | 14.8            |
| Same heated 2 hours at 100° C.....        | 14.0               | 12.5    | 15.4            |

The above data clearly shows that the new magnesium-calcium alloy is readily hardened without elaborate heat treatment to a value equal to or better than that of antimonial lead grid metal, the latter in turn being superior to the calcium-lead alloy. Conventional lead cable alloys, containing, e. g., 1% antimony or 2% tin, are too soft to merit comparison.

## Tensile strength (Lbs./Sq. In.)

| Material tested                   | Lead alloyed with— |         |       |                 |
|-----------------------------------|--------------------|---------|-------|-----------------|
|                                   | 8% Sb              | .03% Ca | 3% Sn | .03% Mg-.05% Ca |
| Cold rolled strip.....            | 4,800              | 5,200   | 3,100 | 5,000           |
| Above aged 2 months at 30° C..... | 4,500              | 5,800   | 3,100 | 6,200           |
| Same heated 1 hour at 100° C..... | 4,200              | 5,900   | 3,100 | 7,600           |

The superior strength of the rolled lead-magnesium-calcium sheet metal is quite evident from the above data and the high strength values developed by simply aging a rolled strip, either at room or an elevated temperature, are quite remarkable.

## Composition stability

In almost any process in which metal is cast there is always a certain amount of material in

the nature of risers, gates, spillage and spoilage which must be returned to the process without special treatment or material loss if reasonably low costs are to be obtained. In the manufacture of storage battery grids the weight of material that must be remelted commonly approximates the weight of satisfactory grids produced but fortunately ordinary antimonial grid metal can be repeatedly remelted without a very great change in composition. This is illustrated by the following test in which grid metal analyzing 7.83% Sb and 0.222% Sn was tested in a special machine equipped with a revolving paddle which swept the surface of the molten metal (temperature 355° C.) at exactly 100 R. P. M. for 10 minutes. At the end of the test the composition analyzed 7.77% Sb and 0.215% Sn. Applying the same test to a calcium-lead alloy containing initially .047% calcium, the calcium content dropped to .023% which represented a loss of 50% of the vital alloying constituent. However, when the test was applied to a calcium-magnesium-lead alloy of the present invention which contained .047% Ca and .020% Mg, the calcium and magnesium contents were only very slightly affected—the final metal analyzing .045% Ca and .018% Mg. Similarly, a calcium-magnesium-lead alloy modified with tin (.05% Ca, .02% Mg, .26% Sn) was remelted and cast twice with no detectable change in composition, while a calcium-lead alloy suffered a decrease in its calcium content from .05% down to .005% with the same treatment.

#### Fatigue properties

The following table illustrates the fatigue properties of several typical lead alloys as compared with the magnesium-calcium-lead alloy of the invention modified with tin:

| 40 | Composition                               | Fatigue strength;<br>(lbs./sq. in.) |
|----|-------------------------------------------|-------------------------------------|
| 41 | 0.06% Cu, balance Pb.                     | 780                                 |
| 42 | 8.0% Sb, balance Pb.                      | 1,000                               |
| 43 | 0.038% Ca, balance Pb.                    | 1,400                               |
| 44 | 0.32% Sn, .045% Ca, .026% Mg, balance Pb. | 2,200                               |

All tests were for 20,000,000 reversals on a rotating beam machine at 2,000 R. P. M.

#### Creep tests

The following creep data were obtained from tests conducted at room temperature for periods of from 1 to 4 years and illustrate the marked superiority of the magnesium-calcium base alloys to all others:

| 60 | Lead alloyed with—   | Time to creep 1%<br>Days | Load (lbs./sq.<br>in.) |
|----|----------------------|--------------------------|------------------------|
| 61 | 2% Sn.               | 350                      | 190                    |
| 62 | 1% Sn.               | 175                      | 233                    |
| 63 | 10% Sb.              | 220                      | 232                    |
| 64 | 0.06% Cu.            | 240                      | 437                    |
| 65 | 0.13% Ca.            | 1,200                    | 578                    |
| 66 | 0.03% Ca.            | 290                      | 700                    |
| 67 | 0.045% Ca, 0.03% Mg. | More than 1,200          | 732                    |

#### Corrosion resistance

Corrosion resistance of any series of alloys is very difficult to evaluate because an alloy that is

superior in one particular set of circumstances may be inferior in another. For instance, in battery strength sulphuric acid a lead alloy containing .04% Mg and .05% Ca was found to have excellent corrosion resistance as measured by loss in weight but suffered from a peculiar penetration of the alloy in about 3 months' time when the temperature was raised to 70° C. However, this difficulty was completely avoided by adding 0.25% tin to the alloy with no loss in physical properties. A lead alloy containing .03% Mg, .04% Ca and .25% Sn was found to be equal to regular 8% antimony grid metal in general corrosion resistance and superior to it for battery purposes due to the former's freedom from the evils of sulphation and galvanic action which accompany the use of antimonial lead grid metal. For cable purposes the use of the calcium-magnesium-lead base metal modified with either copper or tin is recommended since certain brands of lead now on the market contain a desirable amount of the fourth metal, e. g., lead-copper alloy containing 0.06% of the latter element. Such leads are generally used for acid exposures. For other specific purposes other additions may be made within the scope of the invention.

From the data herein adduced, it will be readily apparent that the alloys of the invention possess and exhibit properties which ideally fit them for numerous uses. Accordingly, while their value has been specifically mentioned with reference to grid metal and cable sheathing, it will be understood that they may be successfully utilized in many other fields.

The alloy compositions of the invention may be readily compounded by conventional processes employed by those skilled in the art for producing other lead alloys, as, for example, by simply incorporating the requisite amounts of the alloying constituents in a proper quantity of molten lead without any particular regard to the sequence of their addition. Once compounded, the new alloy compositions can be manufactured into cable sheathing, battery grids and other products by methods well known in the respective arts.

#### What is claimed is:

1. An alloy consisting of 0.01% to 0.3% magnesium, 0.01% to 0.1% calcium, 0.03% to 3% of a corrosion resistant constituent selected from the group consisting of cadmium, copper, mercury and tin, and the balance lead.
2. An alloy consisting of 0.01% to 0.1% calcium, 0.01% to 0.3% magnesium, cadmium not exceeding 3%, and the balance lead.
3. An alloy consisting of 0.01% to 0.1% calcium, 0.01% to 0.3% magnesium, copper not exceeding 3% and the balance lead.
4. An alloy consisting of 0.01% to 0.1% calcium, 0.01% to 0.3% magnesium, tin not exceeding 3%, and the balance lead.
5. A cable sheath containing about 0.01% to about 0.1% calcium and about 0.01% to about 0.3% magnesium, the balance being substantially all lead, characterized by marked resistance to both fatigue and creep.

JESSE O. BETTERTON.

ALBERT J. PHILLIPS.

ALBERT A. SMITH, JR.